

3,202,579

## PHOSPHINIC ACID DERIVATIVES FOR PROTECTION OF HAIR FROM DAMAGE IN BLEACHING AND DYEING THE SAME

Peter Berth, Dusseldorf-Benrath, and Günter Reese, Dusseldorf, Germany, assignors to Therachemie Chemisch Therapeutische Gesellschaft m.b.H., Dusseldorf, Germany

No Drawing. Filed Sept. 19, 1963, Ser. No. 310,165  
Claims priority, application Germany, Mar. 2, 1963,

T 23,551

5 Claims. (Cl. 167—83)

The invention relates to agents which prevent or, at least minimize, damage to hair, particularly human hair, when subjected to bleaching and dyeing operations.

For the purpose of dyeing and bleaching of hair, oxidizing substances have long been used, such as hydrogen peroxide, percarbamide, perborate, persulfate and other compounds emitting active oxygen. It is a well known fact that that oxidizing treatment, aside from destroying pigments in the hair, also attacks the fibrous substance of the hair itself. The damage thus inflicted manifests itself, e.g., in an increased alkali solubility and in a decrease of the mechanical properties of the hair, e.g., a strong decrease in its tear resistance, diminishing gloss and grip and increasing brittleness.

It now has been found that damage to hair upon bleaching and dyeing with active oxygen can largely be averted when the agents hereinafter described are employed. These agents are characterized by a content of compositions having the following formulae:



wherein X represents either —OH or —NH<sub>2</sub>; R<sub>1</sub> is an aryl radical or an aliphatic radical having 1 to 5 carbon atoms, or the radical



and wherein R<sub>2</sub> and R<sub>3</sub>, respectively, denote individually, in Formula 1 as well as in Formula 1a, a hydrogen atom or an alkyl radical having 1 to 5 carbon atoms. Also applicable, in lieu of the compounds shown as (1) and (1a), respectively, are their water-soluble salts. Compounds of the composition (2), which is one embodiment of Formula 1 above,



can be produced by several methods known per se. For instance, phosphorous acid can be reacted with carboxylic acid chlorides or carboxylic acid anhydrides or with mixtures of both such compounds to yield these compounds. Readily available in large scale production are reaction products of phosphorous acid with acetyl chloride and/or acetic anhydride. Finally, in lieu of the carboxylic acid chlorides and phosphorous acid, phosphorous trichloride and carboxylic acids can be used in suitable stoichiometrical proportions. Depending on the method of production, pure single products or mixtures of pure products are obtained.

Instead of the acid reaction products named in the

formulae above, frequently their corresponding alkali salts, e.g., sodium, potassium, ammonium salts, and also their ethanolamine salts are used in practice, which are produced by neutralization of the acids. Likewise, the water-soluble esters are suited for the purpose at hand, produced by partial esterification of the hydroxyl groups with methanol, ethanol, propanol, butanol or amyl alcohol.

Production of the compounds named above having the Formula 3, another embodiment of Formula 1 above, i.e.,



is accomplished by the reaction of phosphorus trihalides with organic nitriles or with malonic acid dinitrile, respectively, whereby substantially 2 mols PCl<sub>3</sub> are to be applied to each mol nitrile. The reaction product then is hydrolyzed to the free acid which, subsequently, can be converted into the corresponding salts or esters, as above.

The compounds named above can be used singularly or as mixtures of the different substance named.

According to the invention, the materials named can be employed on carrier substances or can be admixed to a solution, a gel, a cream or a powder, or else they may be used in combination with the oxidizing agent. Furthermore, they can be incorporated in a treating agent, such as a rinse or a hair wash. The damage-preventing substances are applied in quantities of 0.01 to 10 percent by weight, calculated on the agent in which incorporated, and preferably in amounts of 0.1 to 2 percent by weight. If desired, larger amounts can be used, although this does not have any practical advantages.

The hair treating agents containing the damage-preventing substances also may contain, if desired, further customary additives, such as perfume oils, dyestuffs, thickeners, fatty alcohols, anionactive and cationactive and nonionic wetting agents. Particularly suitable thickeners are cellulose derivatives, polyvinylpyrrolidone, polyacrylates, alginates and, in certain instances, fatty alcohols. Suitable wetting agents include fatty alcohol sulfates, alkyl sulfates and condensation products of fatty alcohols with ethylene oxide, whereby the alkyl radical in all instances has a chain length of 12 to 18 carbon atoms. Also usable are alkylbenzenesulfates and alkylpyridinium salts.

Hair treated with the agents according to the invention are distinguished by high gloss, improved hand or grip and especially good elasticity, as compared to hair which had been treated in the usual manner under equal conditions. The difference in damage to the hair becomes evident from the following examples, wherein this is expressed numerically by the differences in alkali solubility and stretch or elongation. It should, however, be pointed out that these examples are given merely by way of illustration, not of limitation, and that numerous changes may be made in the details without departing from the spirit and the scope of the invention as hereinafter claimed.

### EXAMPLE 1

As hair bleach, a 6 percent H<sub>2</sub>O<sub>2</sub> solution was employed in each instance whose pH was adjusted to 10 with ammonia shortly before application. Table 1 below shows, in the second column, the duration of the reaction period in minutes. Upon bleaching with the agents according to the invention (method 2, first column), the H<sub>2</sub>O<sub>2</sub> solution furthermore contained 0.1 percent of a reaction product of phosphorous acid of the Formula 4:



This substance had been produced according to the process disclosed in JACS 34, 492-499. The alkali solubility of the hair, expressed in percent by weight, was determined according to the method of H. Freytag, Parfumerie und Kosmetik 41, Nr. 10, (1960), 405 (a German publication). The alkali solubility of entirely untreated hair lies between 2 and 6 percent.

Table 1  
ALKALI SOLUBILITY<sup>1</sup>

| Method | Treating Time (minutes) | Kind of Hair <sup>2</sup> |      |      | Average Alkali Solubility, percent |
|--------|-------------------------|---------------------------|------|------|------------------------------------|
|        |                         | A                         | B    | C    |                                    |
| 1      | 30                      | 12.2                      | 11.7 | 12.0 | 12                                 |
| 2      | 30                      | 9.3                       | 8.7  | 9.4  | 9                                  |
| 1      | 120                     | 31.7                      | 33.7 | 22.6 | 29                                 |
| 2      | 120                     | 19.6                      | 15.8 | 14.1 | 17                                 |

<sup>1</sup> Alkali solubility was determined by a one-hour exposure of the hair at 65° C. in 0.1 n NaOH (aqueous), expressed in percent by weight.

<sup>2</sup> A, B and C denotes hair of three different persons.

### EXAMPLE 2

Hair was bleached with  $H_2O_2$  solutions of the composition as in Example 1 for 120 minutes. The softening coefficient ( $K_E$  value) then was determined according to J. Mimra (Parfumerie und Kosmetik 42, Nr. 7, 253-360). The  $K_E$  values increase with growing damage to the hair. The softening coefficient, an average of 40 individual determinations of untreated and conventionally bleached hair, was 7.8, as compared to that after a treatment with solutions containing an additive consisting of the Formula 4 given in Example 1, which had a softening coefficient of 4.9.

### EXAMPLE 3

8 parts by weight fatty alcohol and 7 parts by weight of a fatty alcohol sulfate (chain length of both 16 to 18 carbon atoms), and one part by weight fatty alcohol (chain length 12 to 14 carbon atoms) were heated to a melt at 80° C. and emulsified with 34 parts by weight water at that temperature. The cream obtained after cooling was adjusted to a pH of 10.0 by addition of 4 parts by weight concentrated ammonia and made up to 100 parts with water. For the purpose of bleaching human hair blond, 30 g. of a mixture of 28 g. melamine perhydrate and 2 g. 1-aminobenzyl-1,1-diphosphonic acid in the form of its sodium salt were stirred into 100 g. of the cream, and this mixture evenly distributed on the hair to be bleached. Hair thus rendered blond distinguished itself by particular elasticity and mechanical qualities which by far surpassed average values.

Equally good results were obtained by adding initially to the cream 2 g. 1-aminobenzyl-1,1-diphosphonic acid or 2 g. hydroxybenzyl-1,1-diphosphonic acid in the form of their sodium salts.

### EXAMPLE 4

An agent for bleaching hair blond was prepared by dissolving

Parts of the condensation product of stearyl alcohol with 8 mols ethylene oxide 30  
Parts paraffin oil 20  
Parts glycerol 10  
Parts concentrated aqueous ammonia 4  
Parts water 36

(all parts by weight) and stirring to a homogeneous mass. The transparent and highly viscous mass thus obtained was mixed with 5 g. sodium perborate and 0.2 g. 1-aminoethane-1,1-diphosphonic monomethyl ester. The hair bleached therewith had good elasticity and good hand or grip.

### EXAMPLE 5

A hair bleaching agent in powder form was produced

by mixing 25 parts by weight alkyl sulfate, 50 parts by weight seda, 20 parts by weight sodium persulfate and 5 parts by weight of the compound having the Formula 5:



(5)

in the form of its sodium salt, whereby X selectively denotes, with equally good result, either  $-\text{NH}_2$  or  $-\text{OH}$ . Damage to the hair upon bleaching with such a product is reduced to a considerable extent as compared to an equal treatment but without the reaction product of phosphorous acid.

### EXAMPLE 6

For dyeing of hair, 100 parts by weight of a dyeing cream on the basis of customarily used oxidation dyes are mixed, shortly before application, with a solution of 0.2 part by weight of the reaction compound of phosphorous acid, Formula 4 (see Example 1) in 30 parts by weight of 6 percent aqueous  $H_2O_2$ .

Hair dyed with this mixture has exceptional gloss and grip. The rate of damage to the hair is considerably less than that when the reaction product of phosphorous acid is omitted from the otherwise like agent.

### EXAMPLE 7

A bleaching agent was produced in liquid form by dissolving 1 part by weight of a compound having the Formula 6:



(6)

in form of its ethanolamine salt in 80 parts by weight 10% aqueous  $H_2O_2$ . The pH was adjusted to 10 by further addition of ethanolamine, and the solution made up to 100 parts with water. The damage to the hair upon treatment with this agent was ostensibly less than that treated with a comparative bleach of the same composition but without the diphosphonic acid derivative.

Practically the same result was obtained when, as additive the compound having Formula 7 was used under otherwise the same conditions:



### EXAMPLE 8

Prior to bleaching, the hair was rinsed with a solution containing 10 parts by weight of compound Formula 4 (see Example 1), in the form of its potassium salt, and 10 parts by weight cetyltrimethylammoniumchloride per 100 parts by weight water. Thereafter, bleaching was carried out in the customary manner with an  $H_2O_2$  solution. The hair thus treated exhibited considerably better elasticity than hair which had not been rinsed with the above solution prior to bleaching in the same manner.

What is claimed is:

1. A composition for the prevention of damage to hair upon dyeing and bleaching and for the improvement of gloss, elasticity and grip of said hair, comprising substances selected from the group consisting of at least one oxidizing dye, a bleach, and mixtures thereof, plus 0.01 to 10 percent of a substance selected from the group consisting of phosphonic acid derivatives, their water-soluble methanol, ethanol, propanol, butanol, and amyl alcohol esters, and their sodium, potassium, ammonium, and

ethanolamine salts; said phosphonic acid derivatives having the formula



wherein  $\text{R}_2$  and  $\text{R}_3$  individually are selected from the group consisting of hydrogen and an alkyl having 1 to 5 carbon atoms;  $\text{X}$  is selected from the group consisting of  $-\text{OH}$  and  $-\text{NH}_2$ ; and  $\text{R}_1$  is selected from the group consisting of phenyl, a saturated aliphatic group having 1 to 5 carbon atoms, and the group having the configuration



2. A process for the prevention of damage to hair upon bleaching and dyeing with oxidizing dyes and for the improvement of gloss, elasticity and grip of said hair, which comprises rubbing into said hair, substantially at room temperature, a composition consisting of a carrier plus 0.01 to 10 percent by weight of a compound selected from the group consisting of phosphonic acid derivatives, their water-soluble methanol, ethanol, propanol, butanol, and amyl alcohol esters, and their sodium, potassium, ammonium, and ethanolamine salts; said phosphonic acid derivatives having the formula



wherein  $\text{R}_2$  and  $\text{R}_3$  individually are selected from the group consisting of hydrogen and an alkyl having 1 to 5 carbon atoms;  $\text{X}$  is selected from the group consisting of  $-\text{OH}$  and  $-\text{NH}_2$ ; and  $\text{R}_1$  is selected from the group consisting of phenyl, a saturated aliphatic group having 1 to 5 carbon atoms, and the group having the configuration



3. The process as defined in claim 2, wherein said compound is dispersed in a bleaching cream.  
 4. The process as defined in claim 2, wherein said compound is incorporated in a dyeing and bleaching solution.  
 5. The process as defined in claim 2, wherein said compound is dissolved in a hair rinse and is applied to the hair prior to the bleaching and dyeing step.

#### References Cited by the Examiner

##### FOREIGN PATENTS

321,397 6/57 Switzerland.

##### OTHER REFERENCES

Leibig's Annalen der Chemie, vol. 623, page 103 (1953).

35 JULIAN S. LEVITT, Primary Examiner.